

## UNITED STATES PATENT OFFICE

2,564,659

## RE-ETCHING ELECTROTYPE

John Lomax, Kew Gardens, N. Y., assignor to  
Electrographic Corporation, New York, N. Y.,  
a corporation of Delaware

No Drawing. Application November 6, 1948,  
Serial No. 58,789

2 Claims. (Cl. 41—42)

1

The present invention relates to a novel and improved process of improving the printing quality of electrotypes and other duplicate printing plates.

Objects and advantages of the invention will be set forth in part hereinafter and in part will be obvious herefrom, or may be learned by practice with the invention, the same being realized and attained by means of the processes, steps and combinations pointed out in the appended claims.

The invention consists in the novel steps, processes, compositions and improvements herein shown and described.

The present invention has for its object the provision of a novel and improved process of improving the quality of duplicate printing plates, such as electrotypes. A further object is the provision of a process by which the printing characteristics or tone quality of electrotypes may be corrected as desired so that the electrotypes are more suitable for printing as part of a four color set to be printed at high speed on rotary web presses having a common impression cylinder. Another object is the provision of a process of opening up the shadow dots in a color printing plate so that the ink to be printed by such plate will trap better.

In high speed rotary, letterpress color printing, the colors last to be printed often show serious picking in the full tone or shadow areas as the etched portions between the halftone dots are not sufficiently deep in the duplicate originals or electrotypes as supplied to the printer, usually due to the original plates having been produced for printing at lower speeds or on older types of printing presses. According to the present invention, a process is provided for locally etching one or more of the plates of the color set, so that the spaces between the halftone dots are deepened to provide for better trapping of the ink as a wet color is laid on the still wet color printed by a previous plate.

According to the present invention, the duplicate original or electrotype still bearing the thin film of silver which formed the conductive portion of the mold in which it was deposited has the tops of the dots covered by a thin uniform film of a mordant-resistant ink, such as a "topping ink." The recessed areas of the plate, that is the spaces between the dots, are then filled by rubbing the surface of the plate with a relatively inert, fine powder of a light and preferably white color, thus revealing the tone values of the plate and also serving to influence the subsequent etching operation.

2

Thereafter, the plate is heated moderately to about 200° F. so as to cause the topping ink to flow slightly and insure that the film of ink covers the tops of the dots without any pinholes or other unevenness. The fine powder filling the recesses in the plate also serves to prevent the topping ink while soft from flowing into the recesses or from coating the side walls of dots so as to interfere with the etching operation.

10 The plate is then placed face up on a cold, flat stone, at room temperature, or other heat absorbing surface, and its surface is covered by a film of ferric chloride etching solution, such as is commonly used for etching of copper in photoengraving. This layer or film of solution is preferably as thick as can be conveniently and easily held on the plate without damming the edges of the plate and is usually from  $\frac{1}{2}$  to  $\frac{1}{16}$  inch. The etching solution is allowed to remain on the plate 15 from 4 to 10 minutes, until the plate has been opened up to the desired extent.

During the etching action, uniformity of etching is secured and excessively rapid etching is prevented by maintaining the plate cold due to the 20 withdrawal of the heat generated by the etching by the heavy stone on which the plate is supported. When the etching has been sufficiently accomplished, the etching solution is rinsed off in running water which also removes the powder, 25 the surface of the plate is dried and powder is again applied so that the plate may be judged as to its tone value. If satisfactory, the topping ink is removed by solvent and the powder is brushed out of the recesses preparing the plate for curving 30 and printing.

If desired, only a portion of the plate may be etched and such control is exercised by staging the plate prior to etching. Thus, the areas which do not need etching may be covered with asphaltum or staging ink by means of a brush, as is 35 done in photoengraving.

It will be understood that the foregoing general description and the following detailed description as well are exemplary and explanatory of the invention but are not restrictive thereof.

Referring now in detail to the present preferred and illustrative manner of carrying out the process of the invention, the plates which are particularly useful and to which the process is particularly adapted are duplicate original letterpress printing plates for halftone color reproduction, such as solid copper electrotypes produced from plastic molds which bear on their printing face an extremely thin (usually much less than 50 0.0001") layer of silver. This silver was origi-

nally chemically deposited in the plastic mold and served to form the conductive face of the mold during the electrodeposition process. Such duplicate plates are customarily used in high speed rotary printing rather than original plates, as they substantially duplicate the original plates and can be made in quantity sufficient to accommodate the needs of advertisers and others so that impressions can be run on different printing presses.

However, most printing plates for letterpress halftone are etched so as to be particularly adapted for printing where one or two colors are printed and the third and fourth colors are printed at a later time, sometimes only a few seconds later but often days later. During the time intervening between the printing of the first two and the last two colors of a four-color reproduction, a sufficient amount of time elapses to allow the first two colors to set or be absorbed slightly by the paper so that printing of the third and fourth colors are facilitated. However, in the latest type of printing equipment the four colors are usually printed in rapid succession so that the total time required for the printing of the four color plates is at most only one second or less. In such type of printing it is found that the quantity of ink laid on the paper by the first two plates is so great that the ink carried by the third and fourth plates and which should print in superposition on the first and second impressions does not trap properly and the quality of the impressions is not as good as expected.

According to the present invention, the plates, or some of them to be printed in this manner are treated so as to increase the depth of the recesses between the dots, particularly in the full-tone and shadow areas of the plate, without greatly reducing the area of the dots which would correspondingly change the intensity of the tone printed by that portion of the plate. The finished duplicate electrolyte still bearing the silver layer on its printing face is placed on a flat surface and is lightly inked by means of a relatively hard inking roller, and for this purpose the inking roller is charged with a "topping ink" which is a relatively soft, acid resistant ink which can be applied to the tops only of the dots and will form an acid-resistant film thereon. The plate is then powdered with some relatively inert non-abrasive powder of a light color, such as magnesia so that the recesses of the plate are filled. When the excess powder has been removed, the plate is gently heated to a uniform temperature of about 200° F. which causes the topping ink to soften and flow slightly thereby insuring that the tops of the dots are uniformly covered without pin-holes, which would cause the printing surface of the plate to be injured during the etching operation.

After this mild burning-in operation, the plate is cooled and placed on a relatively cold, flat, heat-absorbing surface such as a thick, flat stone at room temperature. The upper printing surface of the plate is level and is then flowed with a full strength etching solution of aqueous ferric chloride which is held by the surface of the plate so long as the film or layer of etching solution is not too thick. For this purpose, the layer of solution is usually from  $\frac{1}{2}$  to  $\frac{1}{16}$  inch and is allowed to remain on the printing surface of the plate for a period of from four to ten minutes, or until the plate has been etched sufficiently to deepen the recesses to the desired extent.

The action of the aqueous ferric chloride solu-

tion in combination with the relatively inert powder filling the recesses in the plate serves to moderate the action of the etching solution or mordant, also serves to prevent excessive undercutting of the dots thereby deepening the dots without excessively reducing their area and their printing value. The relatively inert filling powder also serves during the burning-in or heating operation to absorb any of the topping ink which might otherwise flow over the edges of the dots and tend to coat the sides of the dots or run into the bottoms of the recesses. This is particularly important inasmuch as the largest dots receive a correspondingly larger amount of ink due to their greater area and are surrounded by the smallest recesses, while the smallest dots are surrounded by the largest recesses which are also the deepest.

During the etching process, a considerable amount of heat is generated which would impair the resistant qualities of the topping ink and would also accelerate the etching. However, the heat of the etching is quickly dissipated through the copper of the plate to the relatively large mass of stone on which it is supported thereby keeping the plate at a substantially constant temperature during the etching process.

When the etching process has proceeded sufficiently, the plate is quickly rinsed in running water, which not only removes the ferric chloride etching solution, but also washes out the magnesia from the recesses of the printing face of the plate. The plate is then dried and again powdered with the light colored powder so that its printing quality may be judged by the etcher and if the desired correction has been accomplished, the plate is again washed and topping ink is removed from the printing surface by means of a solvent, such as xylol, thereby rendering the plate ready for curving and placing on the press for the printing operation.

The result of the etching process thus carried out is to increase the depth of the recesses between the halftone dots and to slightly reduce the area of the fulltone and shadow dots so that the ink to be carried by them will properly trap with the previously printed colors.

If desired to treat only certain portions of the plate in the manner of the present process, the remainder of the plate may be protected by means of a staging solution, as in photoengraving, such a solution usually being a thin solution of asphaltum dissolved in xylol and applied to the portions of the plate not to be etched by means of a fine brush, this application preferably being made before the application of the topping ink to the printing surface of the plate.

While topping ink is preferred for the rolling up operation, other soft, somewhat thermoplastic and acid or mordant resistant inks which can be uniformly applied may be used. Also, other powders than magnesia may be used, such powders being preferably of a light color to contrast with the surface of the plate, and being of an absorbent and relatively inert character so that they will absorb any flow of excess ink and will not be rapidly acted on by the etching agent. Other mordants or etching solutions than aqueous ferric chloride may also be used so long as their reaction with the metal of the plate does not result in the production of an excessive amount of gas. However, ferric chloride is preferred as it is readily available at a moderate price and the etchers are accustomed to the speed and uniformity of its action.

The silver coating of the plate to be etched is highly desirable as it does not prevent the action of the etching solution, although it does assist the topping ink in forming between them a more effective resist than the topping ink applied directly to the surface of the copper. For this reason, the printer will preferably be supplied with the plates still retaining their silver coating on their printing face, rather than with plates from which the silver has been removed. In this way, the printer may correct the plates to suit his own operation, and this process may be carried out quickly and economically after it has been decided on which type of equipment the plates are to be printed.

The invention in its broader aspects is not limited to the specific processes and steps shown and described but departures may be made therefrom within the scope of the accompanying claims without departing from the principles of the invention and without sacrificing its chief advantages.

What is claimed is:

1. The process of correcting duplicate halftone letterpress plates which comprises lightly rolling up the surface of the plate with a mordant-resistant ink, filling the recesses of the plate with a powder inert with respect to said mordant, heat-

ing the plate and etching the plate with a mordant which generates no gas during etching.

2. A process in accordance with claim 1 in which the plate is a silver-faced copper electro-type; the powder is magnesia; and the mordant is an aqueous solution of ferric chloride.

JOHN LOMAX.

#### REFERENCES CITED

The following references are of record in the file of this patent:

#### UNITED STATES PATENTS

| Number    | Name      | Date          |
|-----------|-----------|---------------|
| 1,592,265 | Gunterman | July 13, 1926 |
| 1,597,443 | Fox       | Aug. 24, 1926 |
| 1,628,857 | Ronning   | May 17, 1927  |
| 1,709,327 | Spalding  | Apr. 16, 1929 |
| 1,903,778 | Conroy    | Apr. 18, 1933 |
| 2,099,697 | Marshall  | Nov. 23, 1937 |

#### OTHER REFERENCES

Smith et al.: Photo-Engraving in Relief, pp. 209-212. Published in 1932 by Pitman & Sons, London.

Clerc: Ilford Manual of Process Work, published by Ilford Lmtd., London, 1946, pp. 220-222.